

## UNITED STATES PATENT OFFICE

2,459,115

## MINERAL OIL COMPOSITION

Edward A. Oberright, Woodbury, N. J., assignor  
to Socony-Vacuum Oil Company, Incorporated,  
a corporation of New York

No Drawing. Application July 6, 1945,  
Serial No. 603,593

6 Claims. (Cl. 252—47.5)

1

This invention has to do in a general way with mineral oil compositions and is more particularly related to compositions comprised of mineral oil and a minor proportion of an added ingredient which will improve the oil in one or more important respects.

It is well known to those familiar with the art that mineral oil fractions refined for their various uses are in and of themselves usually deficient in one or more respects so that their practical utility is limited even in the particular field for which they have been refined. For example, mineral oil fractions refined for use as lubricants have a tendency to oxidize under conditions of use, with the formation of sludge or acidic oxidation products; also, the lighter fractions such as gasoline and kerosene tend to oxidize with the formation of color bodies, gum, etc. In order to prevent the formation of these products and thereby extend the useful life of the oil fraction, it is common practice to blend with such oil fraction an additive ingredient which will inhibit oxidation, such ingredients being known to the trade as oxidation inhibitors, antioxidants, sludge inhibitors, gum inhibitors, etc.

It is also the practice to add other ingredients to mineral oil fractions for the purpose of improving "oiliness" characteristics and the wear-reducing action of such mineral oils when they are used as lubricants, particularly when the oils are used for the purpose of lubricating metal surfaces which are engaged under extremely high pressures and at high rubbing speeds.

Various other ingredients have been developed for the purpose of depressing the pour point of mineral oil fractions which have been refined for use as lubricants. Most refining treatments provide oils containing a small amount of wax which, without the added ingredient, would tend to crystallize at temperatures which render the oil impracticable for use under the low temperature conditions. Additive agents have also been developed for improving the viscosity index of lubricating oil fractions. In the case of internal combustion engines, particularly those operating with high cylinder pressures, there is a decided tendency for the ordinary lubricating oil fractions to form carbonaceous deposits which cause

2

the piston rings to become stuck in their slots and which fill the slots in the oil ring or rings, thus materially reducing the efficiency of the engine. Ingredients have been developed which, when added to the oil, will reduce this natural tendency of the oil to form deposits which interfere with the function of the piston rings.

It has also been discovered that certain types of recently-developed hard metal alloys, such as cadmium-silver alloy bearings, are attacked by ingredients in certain types of oils, particularly oils of high viscosity index obtained by various methods of solvent refining. This corrosive action on such alloys has led to the development of corrosion inhibitors which may be used in solvent-refined oils to protect such bearing metals against this corrosive action.

In the lighter mineral oil fractions, such as those used for fuel purposes, particularly in internal combustion engines, it has been found that the combustion characteristics of the fuel may be controlled and improved by adding minor proportions of various improving agents thereto.

The various ingredients which have been developed for use in mineral oil fractions to improve such fractions in the several characteristics enumerated above are largely specific to their particular applications. Therefore, it has been the practice to add a separate ingredient for each of the improvements which is to be effected.

The present invention is predicated upon the discovery of a group or class of oil-soluble reaction products or compounds which, when added to mineral oil fractions in minor proportions, will improve the oil fractions in several respects.

The novel addition agents contemplated by this invention as multifunctional improvers for mineral oils are oil-soluble, phosphorus-containing and phosphorus- and sulfur-containing reaction products obtained by reacting an aldehyde, a heterocyclic amine and a hydroxyaromatic compound to form a condensation product and thereafter reacting the latter with either: a phosphorus halide to form a phosphorus-containing reaction product; a phosphorous sulfide or thiohalide to form a phosphorus- and sulfur-containing reaction product; or a phosphorus halide, phosphorus thiohalide or a phosphorus sulfide and a sulfurizing material such as elementary

sulfur, a sulfur halide or a mixture thereof to form a phosphorus- and sulfur-containing reaction product. Metal salts of these phosphorus-containing, and phosphorus- and sulfur-containing, reaction products are contemplated herein.

The condensation products obtained by reacting an aldehyde, a heterocyclic amine and a hydroxyaromatic compound are represented by the general formula.



wherein A is an aromatic nucleus, either mono- or poly-cyclic; R' is either hydrogen or an alkyl, aralkyl, alkaryl, aryl, cycloalkyl, alkoxy or aroxy group; a represents the number of R' groups attached to an aromatic nucleus A, and is an integer from 0 to 4; X is a substituent such as an amino, nitro, hydroxyl, carboxyl or halogen group or the like; b represents the number of X groups attached to an aromatic nucleus A and is either 0 or 1; Y is a secondary heterocyclic amine group, attached at a secondary (heterocyclic) nitrogen atom to the carbon atom of a



group; and c represents the number of



groups attached to an aromatic nucleus A and is an integer from 1 to 3. It will be clear that when A is a phenyl nucleus, the sum of a, b, and c will not exceed 5; and when A is a naphthalene nucleus or other polycyclic nucleus, the sum may exceed 5.

Aldehydes contemplated by the present invention are the aliphatic aldehydes, typified by formaldehyde (such as trioxymethylene), acetaldehyde, and aldol (B-hydroxy butyraldehyde); aromatic aldehydes, representative of which is benzaldehyde; heterocyclic aldehydes, such as furfural; etc. The aldehyde may contain a substituent group such as hydroxyl, halogen, nitro and the like; in short, any substituent which does not take a major part in the reaction. Preference, however, is given to the aliphatic aldehydes, formaldehyde being particularly preferred.

The secondary heterocyclic amines are those characterized by attachment of a hydrogen atom to a nitrogen atom in the heterocyclic group. Representative of the amines contemplated herein are morpholine, thiomorpholine, pyrrole, pyrrolidine, pyrrolidine, indole, pyrazole, pyrazoline, pyrazolidine, piperidine, phenoxazine, phenothiazine and their C-substituted analogs. Substituent groups, attached to the carbon atoms of these amines are typified by alkyl, aryl, alkaryl, aralkyl, cycloalkyl, etc. Preferred of these amines is morpholine.

Representative hydroxyaromatic compounds contemplated by the present invention are phenol, resorcinol, hydroquinone, catechol, cresol, xylanol, hydroxyphenyl, benzylphenol, phenylethylphenol, phenol resins, methylhydroxydiphenyl, guiacol, alpha and beta naphthol, alpha and beta methylnaphthol, tolylnaphthol, xylanaphthol, benzylnaphthol, anthranol, phenylmethylnaphthol, phenanthriol, monomethyl ether

of catechol, phenxyphenol, chlorphenol, and the like. Preference in general is to the mono-hydroxy phenols otherwise unsubstituted, particular preference being given to phenol and alpha and beta naphthol.

The hydroxyaromatic compounds may also contain one or more substituent groups such as carboxyl, halogen, nitro, amino and the like; in short, any substituent which does not take a predominant part in the condensation with the aldehyde and the heterocyclic amine. Preferred of such substituents is a carboxyl group.

As indicated hereinabove, the hydroxyaromatic compound may contain one or more alkyl substituents such as short-chain groups, typified by methyl, ethyl, amyl, etc.; or long-chain, relatively high molecular weight hydrocarbon groups having at least twenty carbon atoms, typified by alkyl groups derived from petroleum wax, which is a predominantly straight-chain aliphatic hydrocarbon of at least twenty carbon atoms. It will be obvious to those skilled in the art that the maximum number of alkyl groups is limited by the number of valences on the aromatic nucleus available for substitution. Naturally, the maximum number of such groups which can be attached to a single aromatic nucleus will vary as the nucleus is mono- or poly-cyclic and as the nucleus is otherwise substituted with such groups as carboxy, nitro, amino, halogen and the like.

A typical, and also preferred, alkyl-substituted hydroxyaromatic compound which may be used is a wax-substituted phenol, "wax-phenol." The term "wax" as used herein designates petroleum wax or aliphatic hydrocarbons or hydrocarbon groups of the type which characterize petroleum wax. These so-called "wax" substituents may be obtained by alkylation of the phenol or hydroxyaromatic hydrocarbon with a relatively high molecular weight aliphatic hydrocarbon or mixture of such hydrocarbons (such as petroleum wax) by any suitable alkylation procedure such, for example, as by a Friedel-Crafts condensation of chlorinated petroleum wax with phenol.

The condensation products are believed to be formed in the manner indicated in the following equation, wherein formaldehyde, phenol and morpholine are used as illustrations:



In preparing the condensation products, the reactants may be added to each other in any order. A typical procedure involves adding the aldehyde to an alcohol solution of the hydroxyaromatic compound and the heterocyclic amine. The reaction may also be carried out in the presence of other diluents or solvents such, for example, as benzol, chlorbenzene, tetrachlorethane, mineral oil, etc. In the event that mineral oil is used as a diluent, the mineral oil may be retained, rather than separated from the condensation product, thereby providing a mineral oil concentrate which may be reacted with a phosphorus compound of the type mentioned above, or with such a phosphorus compound and a sulfurizing

material of the type indicated above. Oil concentrates of the phosphorus-containing, and phosphorus- and sulfur-containing, reaction products may be obtained in this manner. Metal salts of these reaction products may similarly be obtained in the form of oil concentrates.

The reaction temperature used in preparing the condensation products may be varied considerably, depending upon the reaction time, the specific reactants used, etc. For example, the reaction can be carried out at 20-25° C. for a relatively long period of time or at the reflux temperature of the reaction mixture over a comparatively short period. By way of illustration, the reactants, in quantities such as shown in the following example, may be thoroughly mixed at 20-25° C. for several hours and the reaction completed at the reflux temperature of the reaction mixture for an additional period of several hours.

The condensation product may be water washed to assure complete removal of any unreacted amine and this is recommended when the amine is high boiling. In general, however, the procedure involves distilling off the solvent which also removes any unreacted amine, water of reaction and water added with the reactants (formaldehyde, for example, is generally used in a 37% aqueous solution).

As indicated hereinabove, the reaction products contemplated herein may be prepared by reacting a condensation product of the type described above with a phosphorus halide, a phosphorus sulfide or thiohalide, or at least one such phosphorus compound and a sulfurizing material. This reaction is preferably carried out in the presence of an inert diluent such as tetrachlorethane, benzene, chlorobenzene, mineral oil, etc. These diluents—except heavy mineral oils—are removed after the reaction by distillation of the reaction mixture which contains the desired reaction product. When a mineral oil is used as the diluent, however, it may be retained, thereby providing a mineral oil concentrate containing the reaction product.

Temperatures of the order of about 20° C. to about 200° C. are generally maintained when reacting a phosphorus halide with a condensation product. The preferred procedure, however, involves adding a phosphorus halide to a condensation product at room temperature (20-25° C.) and thereafter heating the reaction mixture so formed at the reflux temperature of the diluent for several hours. Related phosphorus- and sulfur-containing reaction products, in general, are also prepared under the foregoing conditions by reacting a condensation product with a phosphorus compound and with or without a sulfurizing material.

The phosphorus halides and sulfides which may be used herein are represented by the following:  $\text{PCl}_3$ ,  $\text{POCl}_3$ ,  $\text{PSCl}_3$ ,  $\text{PCl}_5$ ,  $\text{P}_2\text{S}_3$ ,  $\text{P}_3\text{S}_4$ ,  $\text{P}_2\text{S}_5$ ,  $\text{P}_4\text{S}_7$ , etc. Preferred of these materials are  $\text{PCl}_3$  and  $\text{P}_2\text{S}_5$ . While only the phosphorus chlorides are recited above, the corresponding bromides, iodides and fluorides may also be used, but the chlorides are more desirable in view of their lower cost and availability.

As indicated above, the sulfurizing materials are elementary sulfur, sulfur halides and mixtures thereof. Of these materials, sulfur halides are preferred, with sulfur monochloride particularly preferred.

Metal salts of the aforesaid phosphorus-, and phosphorus- and sulfur-, containing reaction products, as indicated above, also fall within the

scope of the present invention. Any metal may be used the oxide or hydroxide of which (in alcohol solution, if necessary) can be reacted with the intermediate condensation product, or a salt of which can be reacted in alcohol solution with the sodium salt of the intermediate product. Among the metals contemplated for this purpose are: copper, beryllium, magnesium, calcium, strontium, barium, radium, zinc, cadmium, mercury, germanium, tin, lead, vanadium, chromium, manganese, iron, cobalt, nickel, ruthenium, palladium, platinum, aluminum, antimony, arsenic, bismuth, cerium, columbium, gallium, gold, indium, iridium, molybdenum, osmium, rubidium, selenium, tantalum, tellurium, thorium, titanium, tungsten, uranium, and zirconium. Preference is given to metals of the alkaline earth group, particularly to barium. As noted above, the metal is preferably introduced by reaction of its oxide or hydroxide with the intermediate condensation product. Where necessary, an alcohol solution of the oxide or hydroxide is used. The metal salts can also be prepared by reacting the sodium salt of the intermediate product with an alcohol solution of a salt of the desired metal, such as stannous chloride, lead acetate, thorium nitrate, titanium tetrachloride, etc.

The phosphorus-containing reaction products are illustrated by the following typical example.

#### EXAMPLE

Fifty grams of wax-phenol (2-18), prepared as described in U. S. Patent No. 2,191,499, and 7.7 grams of morpholine were dissolved in butyl alcohol, and 14.6 grams of Formalin (37%) were added dropwise thereto, addition taking about 20 minutes. The reaction mixture thus obtained was stirred for 2½ hours at room temperature, 20-25° C., and thereafter heated at reflux, 110° C., for 8 hours. Benzol was added to the reaction mixture and was removed therefrom, with butyl alcohol and water of reaction and added water of the Formalin used, by distillation to a maximum temperature of 160° C. at 10 mms. pressure. The reaction product thus obtained was wax hydroxy benzyl morpholine (2-18); nitrogen analysis revealed 1.7% nitrogen, compared with a theoretical nitrogen content of 2.0%.

Thirty grams of wax hydroxy benzyl morpholine (2-18) was blended in 60 grams of mineral oil (S. U. V. of 65 seconds at 210° F.) and heated to 65° C., at which temperature 2.34 grams of  $\text{PCl}_3$  were added dropwise. Tetrachlorethane (200 ccs.) was added in order to provide a uniform reaction mixture. The reaction mixture was then heated at 110° C. for 2 hours. Any HCl present in the form of an HCl-amine complex in the reaction mixture, was removed by washing the reaction mixture with aqueous ammonia, followed with aqueous acetic acid solution and finally with water until the washings were neutral. Tetrachlorethane was removed from the washed-reaction mixture by distilling the latter to a maximum temperature of 175° C. at 10 mms. pressure. The reaction product—Product One—is a 1:2 mineral oil blend and contains 0.58% nitrogen and 0.42% phosphorus.

#### SONCONY-VACUUM TURBINE TEST

Twenty-five cc. samples of a furfural-refined Rodessa crude of S. U. V. of 150 seconds at 100° F. and of blends of this same oil and typical reaction products were subjected to the following test to determine the effectiveness of the reaction products contemplated by this invention as inhibitors for turbine oils: To each sample were

added 1 gram of iron granules and 24 inches of 18 gauge copper wire. The samples were then heated to a temperature of 200° F. with 5 liters of air per hour bubbling therethrough. Two cc. of distilled water were added each day. The results of the tests which were made for color and acidity or neutralization number and amount of sludge formed after certain time intervals are set forth in Table I below.

Table I

| Addition Agent | Per Cent Added | Hours | Lovibond Color | N. N. | Sludge (in mgms.) |
|----------------|----------------|-------|----------------|-------|-------------------|
| None           |                | 162   | 245            | 17.8  | 389               |
| Product One    | 1/4            | 166   | 3              | 0.01  | 2                 |
|                |                | 1,006 | 6              | 0.06  | 24                |
|                |                | 1,345 | 110            | 19.6  | 172               |

## CORROSION TEST

In this test the reaction product was blended with a Pennsylvania solvent-refined oil of S. U. V. of 53 seconds at 210° F., and a section of a bearing containing a cadmium-silver alloy surface and weighing about 6 grams was added to this blend. The oil was heated to 175° C. for 22 hours while a stream of air was bubbled against the surface of the bearing. The loss in weight of the bearing during this treatment measured the amount of corrosion that had taken place. A sample of the straight oil was subjected to the same test at the same time, and the difference between the losses in weight of the two bearing sections demonstrated conclusively the effectiveness of the reaction products contemplated herein as corrosion-inhibitors.

Table II

| Addition Agent | Per Cent Added | Bearing Loss (mgms.) |                 |
|----------------|----------------|----------------------|-----------------|
|                |                | Inhibited Oil        | Uninhibited Oil |
| Product One    | 1/4            | 4                    | 35              |

It will be apparent from the foregoing test data that the characterizing materials of this invention are effective multifunctional oil improving agents.

The improved properties and the degree of improvements effected may be varied with the aldehyde, heterocyclic amine, hydroxyaromatic compound, phosphorus halide or sulfide, and metal used in their preparation and present in the reaction product.

The amount of improving agent used varies with the mineral oil fraction with which it is blended and with the properties desired in the final oil composition. These reaction products, and the metal salts thereof, may be added to mineral oil in amounts of from about 0.01% to about 10%, but amounts of the order of 0.1-5% generally provide satisfactory improvement.

It is to be understood that although I have described certain preferred procedures which may be followed in the preparation of the novel reaction products contemplated herein as multifunctional addition agents for mineral oils and have indicated representative reactants for use in their preparation, such procedures and reactants are merely illustrative and the invention is not to be considered as limited thereto or thereby but includes within its scope such changes and modifications as fairly come within the spirit of the appended claims.

I claim:

1. An improved mineral oil composition comprising a mineral oil having in admixture therewith a small proportion, sufficient to inhibit said oil against the deleterious effects of oxidation, of an oil-soluble, phosphorus-containing reaction product obtained by reacting, at a temperature between about 20° C. and about 200° C., one mol of a phosphorus compound selected from the group consisting of a phosphorus halide, a phosphorus thiohalide and a phosphorus sulfide, with about 2.5 mols of a condensation product represented by the general formula:



wherein A is an aromatic nucleus; R' is selected from the group consisting of hydrogen, alkyl, aralkyl, alkaryl, aryl, cycloalkyl, alkoxy and aroxy groups; a represents the number of R' groups attached to an aromatic nucleus A, and is an integer from 0 to 3; R<sup>2</sup> is selected from the group consisting of hydrogen, alkyl, alkaryl, aralkyl, cycloalkyl and aryl groups; Y is a morpholine group attached at the nitrogen atom thereof to the carbon atom of the



group; and c represents the number of



groups attached to an aromatic nucleus A and is an integer from 1 to 3.

2. An improved mineral oil composition comprising a mineral oil having in admixture therewith a small proportion, from about 0.01 per cent to about 10 per cent, of an oil-soluble, phosphorus-containing reaction product obtained by reacting, at a temperature between about 20° C. and about 200° C., one mol of a phosphorus compound selected from the group consisting of a phosphorus halide, a phosphorus thiohalide and a phosphorus sulfide, with about 2.5 mols of a condensation product represented by the general formula:



55 wherein A is an aromatic nucleus; R' is selected from the group consisting of hydrogen, alkyl, aralkyl, alkaryl, aryl, cycloalkyl, alkoxy and aroxy groups; a represents the number of R' groups attached to an aromatic nucleus A, and is an integer from 0 to 3; R<sup>2</sup> is selected from the group consisting of hydrogen, alkyl, alkaryl, aralkyl, cycloalkyl and aryl groups; Y is a morpholine group attached at the nitrogen atom thereof to the carbon atom of the



65 group; and c represents the number of



75 groups attached to an aromatic nucleus A and is an integer from 1 to 3.

3. An improved mineral oil composition comprising a mineral oil having in admixture therewith a small proportion, sufficient to inhibit said oil against the deleterious effects of oxidation, of an oil-soluble, phosphorus-containing reaction product obtained by reacting, at a temperature between about 20° C. and about 200° C., one mol of a phosphorus halide with about 2.5 mols of a condensation product represented by the general formula:



wherein A is an aromatic nucleus; R' is selected from the group consisting of hydrogen, alkyl, aralkyl, alkaryl, aryl, cycloalkyl, alkoxy and aroxy groups; a represents the number of R' groups attached to an aromatic nucleus A, and is an integer from 0 to 3; R<sup>2</sup> is selected from the group consisting of hydrogen, alkyl, alkaryl, aralkyl, cycloalkyl and aryl groups; Y is a morpholine group attached at the nitrogen atom thereof to the carbon atom of the



group; and c represents the number of



groups attached to an aromatic nucleus A and is an integer from 1 to 3.

4. An improved mineral oil composition comprising a mineral oil having in admixture therewith a small proportion, sufficient to inhibit said oil against the deleterious effects of oxidation, of an oil-soluble, phosphorus-containing reaction product obtained by reacting, at a temperature between about 20° C. and about 200° C., one mol of phosphorus trichloride with about 2.5 mols of a condensation product represented by the general formula:



wherein A is an aromatic nucleus; R' is selected from the group consisting of hydrogen, alkyl, aralkyl, alkaryl, aryl, cycloalkyl, alkoxy and aroxy groups; a represents the number of R' groups attached to an aromatic nucleus A, and is an integer from 0 to 3; R<sup>2</sup> is selected from the group consisting of hydrogen, alkyl, alkaryl, aralkyl, cycloalkyl and aryl groups; Y is a morpholine group attached at the nitrogen atom thereof to the carbon atom of the



group; and c represents the number of



groups attached to an aromatic nucleus A and is an integer from 1 to 3.

5. An improved mineral oil composition comprising a mineral oil having in admixture therewith a small proportion, sufficient to inhibit said oil against the deleterious effects of oxidation, of an oil-soluble, phosphorus-containing reaction product obtained by reacting, at a temperature between about 20° C. and about 200° C., one mol of phosphorus trichloride with about 2.5 mols of a paraffin wax-hydroxy-benzyl morpholine.

6. An improved mineral oil composition comprising a mineral oil having in admixture therewith a small proportion, sufficient to inhibit said oil against the deleterious effects of oxidation, of an oil-soluble, metal- and phosphorus-containing reaction product obtained by reacting, at a temperature between about 20° C. and about 200° C., one mol of a phosphorus compound selected from the group consisting of a phosphorus halide, a phosphorus thiohalide and a phosphorus sulfide, with about 2.5 mols of a condensation product followed by introduction of metal into the phosphorus-containing reaction product so obtained, said condensation product being represented by the general formula:



30 wherein A is an aromatic nucleus; R' is selected from the group consisting of hydrogen, alkyl, aralkyl, alkaryl, aryl, cycloalkyl, alkoxy and aroxy groups; a represents the number of R' groups attached to an aromatic nucleus A, and is an integer from 0 to 3; R<sup>2</sup> is selected from the group consisting of hydrogen, alkyl, alkaryl, aralkyl, cycloalkyl and aryl groups; Y is a morpholine group attached at the nitrogen atom thereof to the carbon atom of the



group; and c represents the number of



50 groups attached to an aromatic nucleus A and is an integer from 1 to 3.

EDWARD A. OBERRIGHT.

#### REFERENCES CITED

55 The following references are of record in the file of this patent:

#### UNITED STATES PATENTS

| Number    | Name           | Date          |
|-----------|----------------|---------------|
| 2,146,584 | Lipkin         | Feb. 7, 1939  |
| 2,263,445 | Reiff          | Nov. 18, 1941 |
| 2,279,218 | Badertscher    | Apr. 7, 1942  |
| 2,282,710 | Dietrich       | May 12, 1942  |
| 2,322,376 | McCleary       | June 22, 1943 |
| 2,334,594 | Zimmer         | Nov. 16, 1943 |
| 2,336,006 | Fuller         | Dec. 7, 1943  |
| 2,339,710 | Lincoln        | Jan. 18, 1944 |
| 2,340,036 | Zimmer         | Jan. 25, 1944 |
| 2,353,192 | Sargent et al. | July 11, 1944 |
| 2,361,957 | Musselman      | Nov. 7, 1944  |
| 2,363,134 | McCleary       | Nov. 21, 1944 |

**Certificate of Correction**

Patent No. 2,459,115.

January 11, 1949.

EDWARD A. OBERRIGHT

It is hereby certified that errors appear in the printed specification of the above numbered patent requiring correction as follows:

Column 3, line 70, for "hydroxyphenyl" read *hydroxydiphenyl*; column 4, line 1, for "phenxyphenol" read *phenoxyphenol*; column 6, line 19, for "si" read *is*; and that the said Letters Patent should be read with these corrections therein that the same may conform to the record of the case in the Patent Office.

Signed and sealed this 14th day of June, A. D. 1949.

[~~SEAL~~]

THOMAS F. MURPHY,  
*Assistant Commissioner of Patents.*